

# UNITED STATES PATENT OFFICE.

RICHARD WITHEY, OF SOUTH BERMONDSEY, ENGLAND.

## TREATMENT OF HIDES.

No. 894,171.

Specification of Letters Patent. Patented July 21, 1908.

Original application filed April 16, 1906, Serial No. 311,954. Divided and this application filed May 27, 1907.  
Serial No. 375,903.

*To all whom it may concern:*

Be it known that I, RICHARD WITHEY, a subject of the King of Great Britain, residing at 103 Verney road, South Bermondsey, in the county of Surrey, England, cycle maker and electrical engineer, have invented certain new and useful Improvements in the Treatment of Hides, of which the following is a specification—that is to say—

0 The invention relates to improvements in the treatment of hides.  
The object of this invention is to produce a leather which will be exceedingly tough and flexible yet inexpensive to produce while at 15 the same time it will be adapted to many purposes to which ordinary leather is inapplicable and more particularly as an armor for pneumatic tires. For this purpose any suitable hide such as ox hide or cow hide is 20 employed and submitted to the following treatment: The raw hide as taken from the animal is soaked in clean water for a period of three to seven days, then blubbered, that is to say, loose pieces of flesh and grease are 25 removed from the flesh side after which it is placed in a pit with a solution of quick lime and water for a similar period, and by this process it is reduced to a gelatinous condition; it is then taken out and unhaired and 30 is then laid in a pit containing a mixture of alum and egg or other suitable albumen for a period of four to ten days after which it is in a condition to be chemically treated.

The alum and egg albumen mixture is 35 composed of 56 lbs. of alum, 4 lbs. of egg albumen and 150 gallons of water and the hides are soaked in this for about four days or longer as circumstances may require. It is then successively placed in each of a series 40 of chemical soaks or baths of graduated strengths, commencing with the weakest, each soak consisting of a combination of sulfuric acid, red arsenic, and sumac liquor in suitable proportions and this soaking is 45 continued for a period of about two days during which period the hide is changed from one soak to another of the next higher gradation as regards strength every twelve hours after which the hide is placed in a soak 50 or bath consisting of a solution of rubber, petroleum benzin, and naphtha for a period of about two days; it is then taken out, strained on stretchers or frames and air dried after which the leather is ready for use.

55 The best way to deal with this part of the

process is to soak the hide in the benzin and naphtha and afterwards to work or knead into it a solution of rubber.

The hide thus treated retains all its natural fibrous and other qualities, has nearly the 60 same flexibility as rubber, is entirely free from grease so that it will readily receive rubber solution and is practically impenetrable with ordinary usage.

In treating say twenty five hides the following proportions may be employed for the 65 principal baths or soaks:

### *The Sumac Soaks.*

|       |                                                      |    |
|-------|------------------------------------------------------|----|
| No. 1 | 150 gallons of water.                                | 70 |
|       | ½ pint sulfuric acid, (specific gravity 1.840.)      |    |
|       | 3 lbs. of red arsenic.                               |    |
| No. 2 | 1 cwt. of sumac.                                     | 75 |
|       | 150 gallons of water.                                |    |
|       | 3 quarts of sulfuric acid, (specific gravity 1.840.) |    |
| No. 3 | 4 lbs. of red arsenic.                               | 80 |
|       | 1½ cwt. of sumac.                                    |    |
|       | 150 gallons of water.                                |    |
|       | 6 quarts of sulfuric acid, (specific gravity 1.840.) |    |
|       | 5 lbs. of red arsenic.                               |    |
|       | 1½ cwt. of sumac.                                    | 85 |

### *The Benzin Soak.*

|                                                                                                                                              |    |
|----------------------------------------------------------------------------------------------------------------------------------------------|----|
| 12 gallons of petroleum benzin.                                                                                                              |    |
| 6 gallons of coal tar naphtha.                                                                                                               |    |
| 56 lbs. of rubber solution of commerce consisting of para rubber 1 lb.; coal tar naphtha ½ gallon; benzol 1 pint and carbon bisulfid ½ pint, | 90 |

or the rubber may be omitted and the hides 95 separately treated therewith as hereinbefore pointed out.

By the means hereinbefore described hides are toughened and rendered flexible and a leather obtained which is practically impenetrable and suitable for many uses to which 100 ordinary leather cannot usefully be put and which can be produced at a trifling increase in cost as compared with existing productions.

I have hereinbefore described the best 105 means that I am at present acquainted with for carrying my invention into effect but I would have it understood that I do not confine myself to the precise details set forth either as regards quantities and periods or 110

116

materials as in practice the former may be somewhat varied and chemical equivalents found for the latter and the following claim must therefore be understood as including 5 such variations.

Having now particularly described and ascertained the nature of the said invention and in what manner the same is to be performed I declare that what I claim is:—

- 10 A process for the treatment of hides consisting in soaking the raw hide taken from the animal in water for a suitable period, about four to seven days for example; then blubbering it, that is removing loose pieces 15 of flesh and grease from the flesh side, then submitting it to the action of lime and water for a similar period; then unhairing it; then steeping it in a mixture of alum and albumen for a suitable period, four to ten days for example; then placing it successively in a se- 20

ries of chemical soaks or baths of graduated strengths each soak consisting of a compound of sulfuric acid red arsenic and sumac liquor for a suitable period, two days for example, and changing said soaks at suitable 25 intervals, every twelve hours for example; then placing the hide in or treating it with a soak or bath of a solution of rubber, petroleum benzin and naphtha for a suitable period, about two days for example; or subsequently treating it with rubber solution and finally straining and air drying the hide substantially as herein shown and described and for the purpose stated.

In witness whereof I have hereunto set my 35 hand in the presence of two witnesses.

RICHARD WITHEY.

Witnesses:

C. H. WHITE,  
F. L. RAND.